

## UNITED STATES PATENT OFFICE.

JOHN P. KEGG, OF PITTSBURGH, PENNSYLVANIA.

## PROCESS OF MAKING ACID-PROOF ALLOYS AND PRODUCT THEREOF.

No Drawing.

Application filed February 28, 1922. Serial No. 539,915.

My invention relates to alloys, and it has for its object to provide an alloy which shall be highly resistant to the action of acids and other corroding agents.

More specifically my object is to provide an acid-proof alloy containing copper and lead, with or without tin, in which relatively large amounts of lead may be used and in which the lead shall be held up and distributed uniformly in the metal.

In making my improved alloys I employ as an agent for preventing segregation of the lead a small amount of an alkali metal, suitably metallic sodium or metallic potassium.

The sodium or potassium are not intended to remain in the final metal. Thus, if sodium is used the final alloy contains substantially no trace of sodium, which apparently volatilizes off while the alloy is being stirred and poured.

One useful alloy which I have made in accordance with this invention may be made by melting the following ingredients in about the proportions specified:

|                 | Parts by weight. |
|-----------------|------------------|
| Copper          | 300              |
| Lead            | 175              |
| Tin             | 25               |
| Metallic sodium | 1                |

which gives a total quantity of 500 parts, the 1 part of sodium being disregarded since it does not remain in the final alloy.

In preparing this alloy, the lead and copper are preferably cleaned thoroughly, and the tin is preferably pure block tin. The copper should be melted first, the lead is then added, then the tin, and finally the sodium, the metal being stirred well during mixing. The melted metal is heated high enough to be very fluid and the alloy is preferably poured as quickly as practicable after the sodium is added.

On analysis, the alloy prepared in the manner just described shows substantially no sodium, but contains the other ingredients in about the original proportions, with only such trifling losses as occur in ordinary foundry practice. Thus, the final alloy may be regarded as having the following approximate composition: copper 60%, lead 35%, tin 5%. This alloy resembles copper in color, but is harder and exceedingly tough, wholly resists the corroding action of sulphuric acid and other acids, and is

homogeneous in structure, the lead being distributed uniformly and held in such a manner that the lead will not segregate or sweat out when the metal is cast or worked.

Another alloy may be made according to this invention by melting together 50 parts by weight of copper and 50 parts of lead, without tin, adding about one part of metallic sodium, and pouring the melt, preferably as soon as possible after the sodium is added. This gives an acid-proof alloy containing approximately 50% of copper and 50% of lead, with the lead held up and distributed uniformly in the metal.

I wish it to be understood that the proportions mentioned above are given only as examples of my process, and that my invention is not restricted to the proportions stated but consists broadly in the use of metallic sodium, metallic potassium or other metallic alkali metal as an agent for producing a homogeneous acid-proof alloy from copper and lead with or without tin. The lead may be present in any proportion up to 50%, or even higher, of the finished alloy. The treatment with sodium or other alkali metal holds up any smaller quantity of lead, and is particularly useful when the lead constitutes 20% to 50% of the alloy. The amount of sodium to be used depends somewhat on the purity of the lead that is used. With very pure lead one part of sodium to 100 parts of the other ingredients is sufficient for my purpose, while with impure lead  $1\frac{1}{2}$  to 2 parts will be required.

I am aware that many attempts have been made to produce alloys of copper, lead and tin, containing large proportions of lead, and that various agents have been added to such alloys for the purpose of distributing the lead and preventing it from segregating as it tends to do is present in any considerable quantity. I am also aware that it has been proposed to add to an alloy of copper, lead and tin a small amount of sodium to increase the fluidity of the alloy and facilitate casting it into small articles. The prior alloy just mentioned, however, makes use of a wholly different material for the purpose of holding up the lead, and the possibility of holding up lead in an alloy of this kind by means of sodium or any other alkali metal has not been recognized prior to my invention.

I am not prepared to state exactly the

manner in which the sodium or potassium acts upon the ingredients of the alloy to make the mixture homogeneous and tough, and I do not wish to be restricted to any theory as to the action of the sodium or potassium. What I know to be a fact is that when sodium or potassium is used in the preparation of an alloy in the manner herein described, the resulting alloy is tougher, more resistant to the action of acids and more homogenous, especially as to the distribution of lead, than the corresponding alloys would be if made without the use of alkali metal.

18 I claim as my invention:

1. The process of making alloys that comprises melting copper and lead together, the lead being present in such quantity as tends to segregate from the other constituents, and 20 adding an alkali metal to the melt, thereby holding the lead in suspension therein.

2. The process of making alloys that comprises melting copper, lead and tin together, the lead being present in such quantity as tends to segregate from the other constituents, and 28 adding an alkali metal to the melt, thereby holding the lead in suspension therein.

3. The process of making alloys that comprises melting copper and lead together, the lead being present in such quantity as tends to segregate from the other constituents, and adding metallic sodium to the melt, thereby holding the lead in suspension therein.

25 4. The process of making alloys that comprises melting copper, lead and tin together, the lead being present in such quantity as tends to segregate from the other constituents, and adding metallic sodium to the melt, 40 thereby holding the lead in suspension therein.

5. The process of making alloys that comprises melting copper and lead together, the lead being present in such quantity as tends 45 to segregate from the other constituents, and adding an alkali metal to the melt, thereby holding the lead in suspension therein, said alkali metal being added in such quantity as not to form a substantial 50 ingredient in the final alloy.

6. The process of making alloys that com-

prises melting copper, lead and tin together, the lead being present in such quantity as tends to segregate from the other constituents, and adding an alkali metal to the melt, 65 thereby holding the lead in suspension therein, said alkali metal being added in such quantity as not to form a substantial ingredient in the final alloy.

7. The process of making alloys that comprises melting copper and lead together, the lead being present in such quantity as tends to segregate from the other constituents, and adding metallic sodium to the melt, thereby holding the lead in suspension therein, 65 said alkali metal being added in such quantity as not to form a substantial ingredient in the final alloy.

8. The process of making alloys that comprises melting copper, lead and tin together, 70 the lead being present in such quantity as tends to segregate from the other constituents, and adding metallic sodium to the melt, thereby holding the lead in suspension therein, 75 said alkali metal being added in such quantity as not to form a substantial ingredient in the final alloy.

9. The process of making alloys that comprises melting a quantity of copper, adding lead to the melted copper, heating the melt 80 sufficiently to make it flow freely, adding a small quantity of an alkali metal to the melt and pouring the mixture immediately after the addition of said alkali metal.

10. The process of making alloys that comprises melting a quantity of copper, adding lead to the melted copper, adding tin to the melted mixture, heating the melt sufficiently to make it flow freely, adding a small quantity of an alkali metal to the melt 90 and pouring the mixture immediately after the addition of said alkali metal.

11. The process of making alloys that comprises melting together substantially 300 parts by weight of copper, 175 parts by 95 weight of lead, and 25 parts by weight of tin, adding to the molten metal approximately 1 part by weight of metallic sodium and then pouring the molten metal.

In testimony whereof, I the said JOHN P. 100 KEGG have hereunto set my hand.

JOHN P. KEGG.